# EUROPEAN PATENT SPECIFICATION

(11) **EP 1 892 732 B1**
(45) Date of publication and mention of the grant of the patent: **13.10.2010**
(21) Application number: 07253320.1
(22) Date of filing: 22.08.2007
(51) Int. Cl.: H01B 7/29, H01B 7/02, H01B 3/44

(54) **Wire and cable insulation**
Draht- und Kabelisolierung
Isolation de fils et de câbles

(30) Priority: 22.08.2006 GB 0616631
(43) Date of publication of application: 27.02.2008
(73) Proprietor: Tyco Electronics UK Limited, Swindon, Wiltshire SN3 5HH (GB)
(72) Inventor: Rodway Giles, Wiltshire SN11 8DJ (GB); Steadman Stuart, Swindon SN5 5RA (GB)
(74) Representative: Beck, Josef

(56) References cited:
- WO-A-2005/119705
- JP-A- 10 340 635
- JP-A- 10 340 639

## Description

The invention relates to wire or cable insulation and methods of manufacture thereof in particular to "zero-halogen'' insulation comprising multiple layers.

In many industries it is essential that wire or cable insulation fulfil exacting requirements as to durability in order to be certified for use in those situations. One example of this is the automotive industry where automotive wiring for use in wiring harnesses is required to be stable upon exposure to high temperatures for considerable periods of time (for instance some automotive wiring insulation must fulfil the "class 3" requirement which requires survival intact for 3000 hours at 125°C). In addition, insulation for automotive wiring is required to be resistant to exposure to the aggressive fluids (such as engine oil and windscreen washer fluid) commonly found in automotive environments. Further, wire and cable insulations for use in the automotive industry must be suitable for contact with an assortment of adhesive and non-adhesive tapes, tubing, connectors, seals and alternative cable jacket materials if the insulation is to be efficiently used in this industry. This is because it is not economically viable to produce wiring harnesses which avoid the use of these components.

There are currently two principle commercial insulation systems for class 3 wiring. Both commercial systems are single wall insulations incorporating polypropylene or cross-linked polyethylene polymers, one variety being low-halogen and the second being zero-halogen.

Low halogen products often contain about 12 wt% bromine as a flame retarding component, combined with diantimony trioxide. However, although this combination is very effective at vapour phase flame retarding, concerns exist over possible effects on the environment of the combustion products of certain halogenated compounds. It is therefore an objective in the wire and cable industry to produce high performance insulation without the inclusion of halogen-containing compounds.

An example of a zero-halogen single wall polypropylene insulation may be found in WO 02/073631 to the applicant, which describes a single layer cable or wire insulation including at least 30 wt% polypropylene homo- and/or copolymer, at least 2 wt% zinc sulphide and/or at least 5 wt% zinc oxide of the whole composition.

Zero-halogen products typically include high levels of hydrated mineral fillers (often from 55 wt% to 60 wt% magnesium hydroxide or aluminium hydroxide). The fillers confer flame retardancy through dilution of the combustible polymer and through loss of the water of hydration during heating or combustion which results in high heat absorbtion. Accordingly, known zero-halogen products overcome the environmental concerns associated with the use of halogenated insulating materials. However, prior to now the exclusion of halogens from the insulating materials has produced insulation with inferior mechanical properties, in particular in terms of insulation abrasion resistance and elongation to break (i.e. the capacity of the insulation to be stretched before it snaps or breaks).

Zero-halogen compounds have also historically suffered from poorer chemical and environmental resistance than halogenated products, and have had difficulty in simultaneously meeting industry standards in terms of electrical and flammability requirements. This is partly because it is easier to meet the standard electrical requirements by reducing the levels of fillers such as magnesium hydroxide or aluminium hydroxide, but more difficult to conform to the flammability standards if this is done.

Accordingly, there is a need in the art for a zero-halogen wire or cable insulation without the drawbacks described above. In particular, it is desirable to develop a zero-halogen insulation which can be used by the automotive industry, in particular in automotive wiring harnesses.

According to the present invention there is provided a zero-halogen wire or cable insulation comprising a non-flame retarded inner layer and a flame-retarded outer layer; the outer layer comprising uncoated magnesium hydroxide.

The invention offers a cost effective cable or wire insulation which can tolerate exposure to high temperatures for long periods of time and exposure to aggressive fluids such as those found within the engine bay (for instance, engine oil or windscreen washer fluid). Further, the wires and cables coated with the inventive insulations can be used in combination with an assortment of adhesive and non-adhesive tapes, tubing, connectors, seals and alternative cable jacket materials. In particular, the presence of the uncoated magnesium hydroxide in the outer layer provides a layer which is highly flame retardant, but inexpensive to produce as it is not necessary to purchase or prepare expensive coated magnesium hydroxide.

The term "zero-halogen'' in the context of this document, is intended to include any insulation with less than 1 wt% halogen. In particular, it is preferred that less than 0.5 wt% halogen be present, more preferably 0.1 wt%, most preferably only trace impurities. In typical embodiments, no halogen-containing compound will be added to a zero-halogen insulation and accordingly any halogen which is present typically arises, purely as a result of impurities in the materials used to form the insulation.

The term 'uncoated' should be regarded as relating to magnesium hydroxide powders which have not been treated to coat the external surface of the powder with a secondary chemical.

According to the present invention, the inner layer shall contain no flame retardant providing an electrical insulator and the outer layer comprises 55 wt% uncoated magnesium hydroxide or greater. This combination of layer composition provides an insulation in which the outer layer is strongly flame retarded and the inner layer is non-flame retarded. This allows the inner layer to meet electrical performance requirements and the outer layer to meet the flammability requirements of the insulation.

The insulation may comprise two-layers only. However, there may be one or more intermediate layers between the inner and outer layer. Where more than two-layers are present, preferably there will be three, four or five layers, more preferably three.

In some preferred embodiments the inner and/or outer layer comprises a polypropylene copolymer. It is often desirable for both the inner and outer layer to comprise polypropylene. Where present, the polypropylene may be a polypropylene homopolymer or copolymer, however, typically the polypropylene will be a polypropylene copolymer. Copolymers are preferred as they offer better flexibility and resistance to elongation. In addition, copolymers typically exhibit better low temperature properties and resistance to cracking than homopolymers.

Where the inner layer comprises polypropylene, it will preferably be present in the range 20-60 wt%, more preferably in the range 25-36 wt%. The inner layer may preferably additionally comprise one or more components selected from 30 - 60 wt% high density polyethylene, 5-15 wt% thermoplastic elastomer, 1-6 wt% antioxidant package, and up to 5 wt% minor ingredients. For instance, the inner layer of the insulation may comprise one or more components selected from 30 wt% polypropylene copolymer, 52 wt% high density polyethylene, 9 wt% thermoplastic elastomer, 4 wt% antioxidant package and up to 5 wt% minor ingredients.

In particularly advantageous embodiments, the inner layer will comprise from 20 - 50 wt% polypropylene, from 30-60 wt% high density polyethylene, 5-15 wt% thermoplastic elastomer, 1-6 wt% antioxidant package, and up to 5 wt% minor ingredients.

Where present, the elastomer improves the flexibility of the insulation thereby reducing the damage resulting from bending the wire during use. The elastomer may, for instance, be an EPDM based elastomer, however the person skilled in the art would understand that many different elastomers could be used in the subject invention.

The types of minor ingredient suitable for use in the invention would be well known to the person skilled in the art and would include, for instance, copper stabilisers (such as zinc sulphide), cross-linking promoters, pigments and processing aids. The stabilisers offer increased compatibility with engine harness components and improve the protection available against the aggressive fluids used in the automotive environment.

The inner layer may be of thickness typical to that of known wire or cable insulations, and will depend upon the gauge of the wire or cable to be protected. However, it is preferred that the inner layer is of thickness in the range 0.1 mm - 0.25 mm. Where a 0.75 mm² gauge primary wire is used, the inner layer will preferably have a thickness of about 0.15 mm, although this thickness would also be appropriate for the protection of wires and cables of other gauges.

In some embodiments the flame-retardant qualities of the outer layer are achieved through the inclusion within the outer layer composition of two or more filler compatible elastomers (for instance, elastomers which are capable of wetting filler particles, thereby facilitating mixing between the filler and the elastomer). Preferably the outer layer will comprise two elastomers, a primary and a secondary elastomer, which will often be present in a weight ratio in the range about 4:1 to about 2:1, preferably about 3:1 primary to secondary elastomer dependent upon the gauge of the wire or cable to be coated. Typically the first elastomer will be the elastomer present in the greatest proportion of the insulation. The combination of the elastomers and the filler offers an outer layer with good mechanical performance, abrasion resistance and low temperature behaviour.

Many different elastomers may be used, as would be understood by the reader skilled in the art. However, it is preferred that each of the primary and secondary elastomer is selected from ethylene propylene elastomer, modified polyethylene resin, polypropylene copolymer, and an ethylene-propylene alloy. In some embodiments, the primary elastomer will be an ethylene propylene elastomer and the secondary elastomer a modified polyethylene resin. The ethylene propylene elastomer imparts improved cold wind performance and the polyethylene resin offers improves the abrasion properties of the layer, and imparts mechanical strength. In alternative embodiments the primary elastomer will be a polypropylene copolymer and the secondary elastomer an ethylene-propylene alloy.

The outer layer may comprise 0-50 wt% polypropylene, preferably 0-20 wt% polypropylene, more preferably from 5-16 wt% polypropylene, in addition to the uncoated magnesium hydroxide flame retardant.

The outer layer may additionally comprise one or more components selected from 6-12 wt% primary elastomer, 3-8 wt% secondary elastomer, 55 - 70 wt% uncoated magnesium hydroxide, 1-6 wt% antioxidant package, and up to 6 wt% minor ingredients. For instance, the outer layer may comprise one or more components selected from 16 wt% polypropylene copolymer, 9 wt% primary elastomer, wt% secondary elastomer, 4 wt% antioxidant package and up to 6 wt% minor ingredients. The minor ingredients incorporated into the outer layer will be similar to those appropriate for inclusion in the inner layer and described above.

In particularly advantageous embodiments the outer layer may comprise 20 - 50 wt% polypropylene, 6 - 12 wt% primary elastomer, 3 - 8 wt% secondary elastomer, 55 - 70 wt% uncoated magnesium hydroxide, 1 - 6 wt% antioxidant package, and up to 6 wt% minor ingredients.

Alternatively, the outer layer may comprise (in addition to polypropylene) one or more components selected from 15-30 wt% ethylene-propylene alloy, 55 - 70 wt% uncoated magnesium hydroxide, 1-6 wt% antioxidant package, and up to 6 wt% minor ingredients. For example, the outer layer may comprise one or more components selected from 5 wt% polypropylene copolymer, 24 wt% ethylene-propylene alloy, 61 wt% uncoated magnesium hydroxide, 4 wt% antioxidant package and up to 6 wt% minor ingredients.

It is often desirable that the outer layer comprise from 0 - 10 wt% polypropylene copolymer, 15-30 wt% ethylene-propylene alloy, 55 - 70 wt% uncoated magnesium hydroxide, 1 - 6 wt% antioxidant package, and up to 6 wt% minor ingredients.

It is preferred that the uncoated magnesium hydroxide (whether present in the outer layer or optionally present in the inner or other layer) has particle size (d90) in the range 3 µm - 40 µm, preferably in the range 10 µm - 20 µm. The most preferred particle size is about 15 µm, a particularly coarse particle size for an inorganic flame retardant that would typically be expected to result in a poor quality insulation, at least in terms of abrasion resistance and stability at high temperature. Known magnesium hydroxide containing insulations typically include magnesium hydroxide of particle size less than 3 µm. However, it has surprisingly been found that the incorporation of relatively coarse particulate matter into the inventive insulations offers an insulation with exceptional properties.

As with the inner layer, the outer layer may be of a range of thicknesses typically used for wire or cable insulations, and will depend upon the thickness of the wire or cable to be covered. As above, however, it is preferred that the outer layer is of thickness in the range 0.1 mm - 0.25 mm. Where a 0.75 mm² gauge primary wire is used, the outer layer will preferably have a thickness of about 0.15 mm, although this thickness would also be appropriate for use with wires and cables of other gauges.

The total combined thickness of the insulation may fall within the range 0.1 mm - 0.5 mm if this is appropriate, preferably in the range 0.2 - 0.35 mm, dependent upon the gauge of the wire to be coated, with the inner and outer layers being present in the ratio 2.5:1 to 1:2.5, preferably in the range 2:1 to 1:2by thickness of layer.

In a second aspect of the invention there is provided a method of manufacture of an insulated wire or cable wherein the insulation is a zero-halogen insulation which comprises at least an inner layer and an outer layer; the outer layer comprising uncoated magnesium hydroxide; the method comprising the step of co-extruding the insulation directly onto the wire or cable.

In a third aspect of the invention there is provided a method of manufacture of an insulated wire or cable wherein the insulation is a zero-halogen insulation which comprises at least an inner layer and an outer layer; the outer layer comprising uncoated magnesium hydroxide; the method comprising the sequential extrusion of the inner layer, the outer layer and any additional intervening layers onto the wire or cable.

So that a stable dual or multi-layer insulation is formed it is preferred that the layers of the insulation form a strong bond during manufacture of the insulation. This bond may be chemical or mechanical or a combination of chemical and mechanical interactions. For instance, the bond could arise during co-extrusion through a low level of mechanical mixing or interdiffusion at the interface between layers. Alternatively, the bond could arise through covalent or intermolecular bonding between layers. The formation of a strong bond between layers is believed to improve the elongation and abrasion resistance of the insulation as the outer layer adopts many of the beneficial mechanical characteristics of the tougher inner layer.

It is to be understood that values given in terms of percentage by weight (wt%) refer to the weight percentage of that component within a given layer unless specifically states as being the weight percentage of the insulation as a whole.

An embodiment of the invention will now be described in detail by way of example only with reference to Figure 1, which is a schematic cross-sectional view through a wire coated with the insulation of the invention.

The insulation of figure 1 covers a single wire 5, although it is equally appropriate for multiple wire or cable applications. There is an inner layer 10 and an outer layer 15, each composed according to one of the specific examples outlined below.

### Examples

### Example 1

An insulation comprising an inner and an outer layer was co-extruded onto a 0.75 mm² gauge wire. The inner and outer layers were each present in a thickness of 0.15 mm.

The inner layer comprised 30 wt% polypropylene copolymer; 52 wt% high density polyethylene; 9 wt% thermoplastic elastomer; 4 wt% antioxidant package; and 5 wt% of the usual minor ingredients including cross-linking promoters, copper stabilisers, pigments and processing aids.

The outer layer comprised 16 wt% polypropylene copolymer; 9 wt% primary elastomer; 5 wt% secondary elastomer; 60 wt% uncoated magnesium hydroxide of mean particle size 15 µm; 4 wt% antioxidant package; and 6 wt% of the usual minor ingredients including cross-linking promoters, copper stabilisers, pigments and processing aids.

The insulated wire is suitable for use as automotive wiring fulfilling the "class 3" requirement which requires survival intact for 3000 hours at 125°C.

### Example 2

An insulation comprising an inner and an outer layer was sequentially extruded onto a 0.75 mm² gauge wire. The inner and outer layers were each present in a thickness of 0.20 mm.

The composition of the inner layer corresponded to that of Example 1, the outer layer comprised 5 wt% polypropylene copolymer; 24 wt% of a catalloy with a MFI of approximately 0.8 (an ethylene-propylene alloy); 61 wt% uncoated magnesium hydroxide of mean particle size 15 µm; 4 wt% antioxidant package; and 6 wt% of the usual minor ingredients including cross-linking promoters, copper stabilisers, pigments and processing aids.

The insulated wire is suitable for use as automotive wiring fulfilling the "class 3" requirement which requires survival intact for 3000 hours at 125°C.

## Claims

1. A zero-halogen wire or cable insulation comprising a non-flame retarded inner layer and a flame retarded outer layer; the outer layer comprising uncoated magnesium hydroxide.

2. An insulation according to claim 1 wherein the level of halogen in any of the layers is less than 1 wt%.

3. An insulation according to claim 1 or claim 2 wherein the inner layer comprises 0 wt% inorganic filler.

4. An insulation according to any preceding claim wherein the outer layer comprises 55 wt% uncoated magnesium hydroxide or greater.

5. An insulation according to any preceding claim wherein there are two layers only.

6. An insulation according to any preceding claim wherein the inner and/or outer layer comprises a polypropylene copolymer.

7. An insulation according to claim 6 wherein the inner layer comprises polypropylene present in the range 20 - 50 wt%, preferably 25 - 35 wt% of the layer.

8. An insulation according to claim 7 wherein the inner layer additionally comprises one or more components selected from 30 - 60 wt% high density polyethylene, 5-15 wt% thermoplastic elastomer, 1 - 6 wt% antioxidant package, and up to 5 wt% minor ingredients.

9. An insulation according to claim 8 wherein the inner layer comprises one or more components selected from 30 wt% polypropylene copolymer, 52 wt% high density polyethylene, 9 wt% thermoplastic elastomer, 4 wt% antioxidant package and up to 5 wt% minor ingredients.

10. An insulation according to any preceding claim wherein the inner layer is of thickness in the range 0.1 mm - 0.25 mm.

11. An insulation according to claim 6 wherein the outer layer comprises polypropylene present in the range 0 - 50 wt%, preferably 5 - 16 wt% of the layer.

12. An insulation according to any preceding claim wherein the outer layer comprises two or more filler compatible elastomers.

13. An insulation according to claim 12 wherein the outer layer comprises a primary and a secondary elastomer, present in a ratio in the range about 4:1 to about 2:1, preferably about 3:1 primary to secondary elastomer.

14. an insulation according to claim 12 or claim 13 wherein each elastomer is selected from ethylene propylene elastomer, modified polyethylene resin, polypropylene copolymer, and an alloy of ethylene and propylene.

15. An insulation according to claim 14 wherein the primary elastomer is an ethylene propylene elastomer and the secondary elastomer is a modified polyethylene resin.

16. An insulation according to claim 14 wherein the primary elastomer is a polypropylene copolymer and the secondary elastomer is an alloy of ethylene and propylene.

17. An insulation according to claims 11 to 16 wherein the outer layer additionally comprises one or more components selected from 6 - 12 wt% primary elastomer, 3 - 8 wt% secondary elastomer, 55 - 70 wt% uncoated magnesium hydroxide, 1 - 6 wt% antioxidant package, and up to 6 wt% minor ingredients.

18. An insulation according to claims 6 to 17 wherein the outer layer comprises one or more components selected from 16 wt% polypropylene copolymer, 9 wt% primary elastomer, 5 wt% secondary elastomer, 4 wt% antioxidant package and up to 6 wt% minor ingredients.

19. An insulation according to claims 6 to 17 wherein the outer layer comprises one or more components selected from 0 - 10 wt% polypropylene copolymer, 15 - 30 wt% alloy of ethylene and propylene, 55-70 wt% uncoated magnesium hydroxide, 1 - 6 wt% antioxidant package, and up to 6 wt% minor ingredients.

20. An insulation according to claim 19 wherein the outer layer comprises, one or more components selected from 5 wt% polypropylene copolymer, 24 wt% alloy of ethylene and propylene, 61 wt% uncoated magnesium hydroxide, 4 wt% antioxidant package and up to 6 wt% minor ingredients.

21. An insulation according to any preceding claim wherein the uncoated magnesium hydroxide has particle size in the range 3 µm - 40 µm, preferably in the range 10 µm - 20 µm.

22. An insulation according to any preceding claim wherein the outer layer is of thickness in the range 0.1 mm - 0.25 mm.

23. An insulation according to any preceding claim wherein the relative thickness ratio of outer layer to inner layer is in the range 2:1 to 1:2.

24. A method of manufacture of an insulated wire or cable wherein the insulation is a zero-halogen insulation which comprises at least an inner non-flame retarded layer and an outer layer; the outer layer comprising uncoated magnesium hydroxide; the method comprising the step of co-extruding the insulation directly onto the wire or cable.

25. A method of manufacture of an insulated wire or cable wherein the insulation is a zero-halogen insulation which comprises at least an inner non-flame retarded layer and an outer layer; the outer layer comprising uncoated magnesium hydroxide; the method comprising the sequential extrusion of the inner layer, the outer layer and any additional intervening layers onto the wire or cable.

## Patentansprüche

1. Halogenfreie Draht- oder Kabelisolierung umfassend eine nicht flammgehemmte Innenschicht und eine flammgehemmte Außenschicht, wobei die Außenschicht unbeschichtetes Magnesiumhydroxid umfasst.

2. Isolierung nach Anspruch 1, wobei die Halogenkonzentration in irgendeiner der Schichten weniger als 1 Gew.-% beträgt.

3. Isolierung nach Anspruch 1 oder Anspruch 2, wobei die Innenschicht 0 Gew.-% anorganische Fülleinlage umfasst.

4. Isolierung nach einem der vorhergehenden Ansprüche, wobei die Außenschicht 55 Gew.-% oder mehr unbeschichtetes Magnesiumhydroxid umfasst.

5. Isolierung nach einem der vorhergehenden Ansprüche, wobei nur zwei Schichten vorliegen.

6. Isolierung nach einem der vorhergehenden Ansprüche, wobei die Innen- und/oder Außenschicht ein Polypropylen-Copolymer umfasst.

7. Isolierung nach Anspruch 6, wobei die Innenschicht Polypropylen umfasst, das in einer Menge im Bereich von 20 - 50 Gew.-%, bevorzugt 25 - 35 Gew.-%, auf die Schicht bezogen, vorliegt.

8. Isolierung nach Anspruch 7, wobei die Innenschicht zusätzlich eine oder mehrere Komponenten umfasst, ausgewählt unter 30 - 60 Gew.-% Polyethylen hoher Dichte, 5 - 15 Gew.-% thermoplastischem Polymer, 1 - 6 Gew.-% Antioxidanspackung und bis zu 5 Gew.-% geringfügiger Bestandteile.

9. Isolierung nach Anspruch 8, wobei die Innenschicht eine oder mehrere Komponenten umfasst ausgewählt unter 30 Gew.-% Polypropylen-Copolymer, 52 Gew.-% Polyethylen hoher Dichte, 9 Gew.-% thermoplastischem Elastomer, 4 Gew.-% Antioxidanspackung und bis zu 5 Gew.-% geringfügigen Bestandteilen.

10. Isolierung nach einem der vorhergehenden Ansprüche, wobei die Innenschicht eine Dicke im Bereich von 0,1 mm - 0,25 mm aufweist.

11. Isolierung nach Anspruch 6, wobei die Außenschicht Polypropylen umfasst, das in einer Menge im Bereich von 0 - 50 Gew.-%, bevorzugt 5 - 16 Gew.-%, auf die Schicht bezogen, vorliegt.

12. Isolierung nach einem der vorhergehenden Ansprüche, wobei die Außenschicht zwei oder mehrere Elastomeren, die mit der Fülleinlage verträglich sind, umfasst.

13. Isolierung nach Anspruch 12, wobei die Außenschicht ein primäres und ein sekundäres Elastomer umfasst, die in einem Verhältnis im Bereich von etwa 4:1 bis etwa 2:1, bevorzugt etwa 3:1 primäres zu sekundäres Elastomer vorliegen.

14. Isolierung nach Anspruch 12 oder Anspruch 13, wobei das Elastomer unter Ethylen-Propylen-Elastomer, modifiziertem Polyethylenharz, Polypropylen-Copolymer und einer Legierung von Ethylen und Propylen ausgewählt wird.

15. Isolierung nach Anspruch 14, wobei das primäre Elastomer ein Ethylen-Propylen-Elastomer und das sekundäre Elastomer ein modifiziertes Polyethylenharz ist.

16. Isolierung nach Anspruch 14, wobei das primäre Elastomer ein Polypropylen-Copolymer und das zweite Elastomer eine Legierung von Ethylen und Propylen ist.

17. Isolierung nach den Ansprüchen 11 bis 16, wobei die Außenschicht zusätzlich eine oder mehrere Komponenten umfasst ausgewählt unter 6 - 12 Gew.-% primärem Elastomer, 3 - 8 Gew.-% sekundärem Elastomer, 55 - 70 Gew.-% unbeschichtetem Magnesiumhydroxid, 1 - 6 Gew.-% Antioxidanspackung und bis zu 6 Gew.-% geringfügigen Betandteilen.

18. Isolierung nach den Ansprüchen 6 bis 17, wobei die Außenschicht eine oder mehrere Komponenten umfasst ausgewählt unter 16 Gew.-% Polypropylen-Copolymer, 9 Gew.-% primärem Elastomer, 5 Gew.-% sekundärem Elastomer, 4 Gew.-% Antioxidanspackung und bis zu 6 Gew.-% geringfügigen Betandteilen.

19. Isolierung nach den Ansprüchen 6 bis 17, wobei die Außenschicht eine oder mehrere Komponenten umfasst ausgewählt unter 0 - 10 Gew.-% Polypropylen-Copolymer, 15 - 30 Gew.-% Legierung von Ethylen und Propylen, 55 - 70 Gew.-% unbeschichtetem Magnesiumhydroxid, 1 - 6 Gew.-% Antioxidanspackung und bis zu 6 Gew.-% geringfügigen Betandteilen.

20. Isolierung nach Anspruch 19, wobei die Außenschicht eine oder mehrere Komponenten umfasst ausgewählt unter 5 Gew.-% Polypropylen-Copolymer, 24 Gew.-% Legierung von Ethylen und Propylen, 61 Gew.-% unbeschichtetem Magnesiumhydroxid, 4 Gew.-% Antioxidanspackung und bis zu 6 Gew.-% geringfügigen Betandteilen.

21. Isolierung nach einem der vorhergehenden Ansprüche, wobei das unbeschichtete Magnesiumhydroxid eine Teilchengröße im Bereich von 3 µm - 40 µm, bevorzugt im Bereich von 10 µm - 20 µm aufweist.

22. Isolierung nach einem der vorhergehenden Ansprüche, wobei die Außenschicht eine Dicke im Bereich von 0,1 mm - 0,25 mm aufweist.

23. Isolierung nach einem der vorhergehenden Ansprüche, wobei das relative Dickenverhältnis von Außenschicht zu Innenschicht im Bereich von 2:1 bis 1:2 liegt.

24. Methode zur Herstellung eines isolierten Drahts oder Kabels, wobei die Isolierung eine halogenfreie Isolierung ist, die mindestens eine nicht flammgehemmte Innenschicht und eine Außenschicht umfasst; wobei die Außenschicht unbeschichtetes Magnesiumhydroxid umfasst; wobei die Methode den Schritt des Coextrudierens der Isolierung direkt auf den Draht oder das Kabel umfasst.

25. Methode zur Herstellung eines isolierten Drahts oder Kabels, wobei die Isolierung eine halogenfreie Isolierung ist, die mindestens eine nicht flammgehemmte Innenschicht und eine Außenschicht umfasst; wobei die Außenschicht unbeschichtetes Magnesiumhydroxid umfasst; wobei die Methode das sequentielle Extrudieren der Innenschicht, der Außenschicht und irgendwelcher zusätzlicher dabei eingeschlossener Schichten auf den Draht oder das Kabel umfasst.

## Revendications

1. Isolation de fils ou de câbles sans halogène comprenant une couche interne non ignifugée et une couche externe ignifugée, la couche externe comprenant de l'hydroxyde de magnésium non enrobé.

2. Isolation selon la revendication 1, dans laquelle la teneur en halogène dans n'importe laquelle des couches est inférieure à 1 % en pds.

3. Isolation selon la revendication 1 ou la revendication 2, dans laquelle la couche interne comprend 0 % en pds d'une charge minérale.

4. Isolation selon l'une quelconque des revendications précédentes, dans laquelle la couche externe comprend 55 % en pds ou plus d'hydroxyde de magnésium non enrobé.

5. Isolation selon l'une quelconque des revendications précédentes, dans laquelle il existe uniquement deux couches.

6. Isolation selon l'une quelconque des revendications précédentes, dans laquelle la couche interne et/ou la couche externe compren(d)(nent) un copolymère de polypropylène.

7. Isolation selon la revendication 6, dans laquelle la couche interne comprend du polypropylène présent dans la plage de 20 à 50 % en pds, de préférence 25 à 35 % en pds de la couche.

8. Isolation selon la revendication 7, dans laquelle la couche interne comprend de manière supplémentaire un ou plusieurs composant(s) choisi(s) parmi 30 à 60 % en pds de polyéthylène haute densité, 5 à 15 % en pds d'élastomère thermoplastique, 1 à 6 % en pds d'un ensemble d'antioxydants, et de jusqu'à 5 % en pds d'ingrédients mineurs.

9. Isolation selon la revendication 8, dans laquelle la couche interne comprend un ou plusieurs composant(s) choisi(s) parmi 30 % en pds de copolymère de polypropylène, 52 % en pds de polyéthylène haute densité, 9 % en pds d'élastomère thermoplastique, 4 % en pds d'un ensemble d'antioxydants et jusqu'à 5 % en pds d'ingrédients mineurs.

10. Isolation selon l'une quelconque des revendications précédentes, dans laquelle la couche interne est d'une épaisseur située dans la plage de 0,1 mm à 0,25 mm.

11. Isolation selon la revendication 6, dans laquelle la couche externe comprend du polypropylène présent dans la plage de 0 à 50 % en pds, de préférence 5 à 16 % en pds de la couche.

12. Isolation selon l'une quelconque des revendications précédentes, dans laquelle la couche externe comprend deux élastomères ou plus compatibles avec la charge.

13. Isolation selon la revendication 12, dans laquelle la couche externe comprend un élastomère primaire et un élastomère secondaire, présents en un rapport situé dans la plage d'environ 4:1 à environ 2:1, de préférence d'environ 3:1 d'élastomère primaire par rapport à l'élastomère secondaire.

14. Isolation selon la revendication 12 ou la revendication 13, dans laquelle chaque élastomère est choisi parmi un élastomère d'éthylène propylène, une résine polyéthylène modifiée, un copolymère de polypropylène, et un alliage d'éthylène-propylène.

15. Isolation selon la revendication 14, dans laquelle l'élastomère primaire est un élastomère d'éthylène propylène et l'élastomère secondaire est une résine polyéthylène modifiée.

16. Isolation selon la revendication 14, dans laquelle l'élastomère primaire est un copolymère de polypropylène et l'élastomère secondaire est un alliage d'éthylène-propylène.

17. Isolation selon les revendications 11 à 16, dans laquelle la couche externe comprend de manière supplémentaire un ou plusieurs composant(s) choisi(s) parmi 6 à 12 % en pds d'élastomère primaire, 3 à 8 % en pds d'élastomère secondaire, 55 à 70 % en pds d'hydroxyde de magnésium non enrobé, 1 à 6 % en pds d'un ensemble d'antioxydants et jusqu'à 6 % en pds d'ingrédients mineurs.

18. Isolation selon les revendications 6 à 17, dans laquelle la couche externe comprend un ou plusieurs composant(s) choisi(s) parmi 16 % en pds de copolymère de polypropylène, 9 % en pds d'élastomère primaire, 5 % en pds d'élastomère secondaire, 4 % en pds d'un ensemble d'antioxydants et jusqu'à 6 % en pds d'ingrédients mineurs.

19. Isolation selon les revendications 6 à 17, dans laquelle la couche externe comprend un ou plusieurs composant(s) choisi(s) parmi 0 à 10 % en pds de copolymère de polypropylène, 15 à 30 % en pds d'alliage d'éthylène-propylène, 55 à 70 % en pds d'hydroxyde de magnésium non enrobé, 1 à 6 % en pds d'un ensemble d'antioxydants, et jusqu'à 6 % en pds d'ingrédients mineurs.

20. Isolation selon la revendication 19, dans laquelle la couche externe comprend un ou plusieurs composant(s) choisi(s) parmi 5 % en pds de copolymère de polypropylène, 24 % en pds d'alliage d'éthylène-propylène, 61 % en pds d'hydroxyde de magnésium non enrobé, 4 % en pds d'un ensemble d'antioxydants et jusqu'à 6 % en pds d'ingrédients mineurs.

21. Isolation selon l'une quelconque des revendications précédentes, dans laquelle l'hydroxyde de magnésium non enrobé a une taille de particule située dans la plage de 3 µm à 40 µm, de préférence dans la plage de 10 µm à 20 µm.

22. Isolation selon l'une quelconque des revendications précédentes, dans laquelle la couche externe est d'une épaisseur située dans la plage de 0,1 mm à 0,25 mm.

23. Isolation selon l'une quelconque des revendications précédentes, dans laquelle le rapport relatif des épaisseurs de la couche externe à la couche interne est situé dans la plage de 2:1 à 1:2.

24. Procédé de fabrication d'un fil ou câble isolé, dans lequel l'isolation est une isolation sans halogène qui comprend au moins une couche interne non ignifugée et une couche externe; la couche externe comprenant de l'hydroxyde de magnésium non enrobé; le procédé comprenant l'étape de co-extrusion de l'isolation directement sur le fil ou le câble.

25. Procédé de fabrication d'un fil ou d'un câble isolé, dans lequel l'isolation est une isolation sans halogène qui comprend au moins une couche interne non ignifugée et une couche externe; la couche externe comprenant de l'hydroxyde de magnésium non enrobé; le procédé comprenant l'extrusion séquentielle de la couche interne, de la couche externe et de toutes couches intermédiaires supplémentaires sur le fil ou le câble.
